# EUROPEAN PATENT SPECIFICATION

(11) **EP 3 362 210 B1**
(45) Date of publication and mention of the grant of the patent: **06.05.2020**
(21) Application number: 16778335.6
(22) Date of filing: 05.10.2016
(51) Int. Cl.: B22F 3/22, C22C 33/02, C22C 38/42, B22F 1/00

(54) **IRON BASED POWDERS FOR POWDER INJECTION MOLDING**
PULVER AUF EISENBASIS FÜR PULVERSPRITZGIESSEN
POUDRES À BASE DE FER POUR UN MOULAGE PAR INJECTION DE POUDRE

(30) Priority: 15.10.2015 EP 15189896
(43) Date of publication of application: 22.08.2018
(73) Proprietor: Höganäs AB (publ), 263 83 Höganäs (SE)
(72) Inventor: LARSSON, Anna, 25657 Ramlösa (SE)
(86) International application number: PCT/EP2016/073721
(87) International publication number: WO 2017/063923

(56) References cited:
- WO-A1-2012/089807
- JOYS J ET AL: "Design of experiments (DOE) study to achieve higher mechanical properties by optimizing particle size distribution and processing parameters of 17-4PH Stainless Steel powder for Metal Injection Molding (MIM).", ADVANCES IN POWDER METALLURGY AND PARTICULATE MATERIALS, 2013, pages FP, 01-9-01-16, XP008179964, Proceedings of the 2013 international Conference on Powder Metallurgy & Particulate Materials sponsored by the Metal Powder Industries Federation
- MURRAY K ET AL: "Effect of particle size distribution on processing and properties of MIM 17-4PH", ADVANCES IN POWDER METALLURGY AND PARTICULATE MATERIALS - 2010, PROCEEDINGS OF THE 2010 INTERNATIONAL CONFERENCE ON POWDER METALLURGY AND PARTICULATE MATERIALS, POWDERMET 2010 - ADVANCES IN POWDER METALLURGY AND PARTICULATE MATERIALS - 2010, PROCEEDI, 2010, XP002756955,

## Description

### FIELD OF THE INVENTION

The present invention concerns an iron-based powder, in particular a stainless steel powder, which is useful for powder injection molding; a composition for powder injection molding; a method of making sintered components from the powder composition; and sintered components made from the powder composition. Using the powder composition it may be possible to obtain sintered parts with densities above 96% of the theoretical density, thus resulting in excellent mechanical properties.

### BACKGROUND OF THE INVENTION

Powder injection molding, also called metal injection molding (MIM) is an interesting technique for producing high density sintered components of complex shapes. In general, fine carbonyl iron powders are used in this process. Other types of powders used are gas-atomized or water-atomized of very fine particle size, the cost of which is relatively high. In order to improve the competitiveness of the MIM process it is desirable to reduce the cost of the powder used. One way of achieving this is by utilizing coarser powders. However, coarse powders have a lower surface energy than fine powders and are thus much less active during sintering. Another issue is that the use of coarse and irregular powders leads a lower packing density and thus the maximal powder content of the feedstock is limited. Lower powder content results in a higher shrinkage during sintering and may lead to, *inter alia,* high dimensional scatter between components produced in a production run.

In a paper by Joys et al. "Design of experiments (DOE) study to achieve higher mechanical properties by optimizing particle size distribution and processing parameters of 17-4PH Stainless Steel powder for Metal Injection Molidng (MIM), published in ADVANCES IN POWDER METALLURGY AND PARTICULATE MATERIALS, 2013, various experiments with feedstocks containing powders having an alloy composition according to 17-4PH material, and catalytic binders, are disclosed. Mechanical properties and sintered densities for sintered components made from the feedstocks, are reported.

WO2012089807 discloses the use of a coarse powder which achieves a theoretical density of more than 95%. There is still a need for technology which can achieve even higher density.

Normally, the solid loading (*i.e.* the portion of iron- based powder) of an iron-based MIM feedstock (*i.e.* the iron- based powder mixed with organic binder ready to be injected) is about 50% by volume, which means that, in order to reach high density after sintering (above 93% of theoretical density), the green component must shrink almost by 50% by volume. This is in contrast to PM components produced through uniaxial compaction which already in green state obtain relatively high density. Therefore, fine powders having high sintering activity are normally used in MIM. By elevating the sintering temperature coarser powders may be used. This, however, results in grain coarsening which in turn gives mechanical properties which are not optimal.

It has unexpectedly been found that a coarse metal powder, wherein the metal powder has a certain composition, can be used in a feedstock for powder injection molding in order to obtain components with a sintered density of at least 96% of the theoretical density.

### SUMMARY

An object of invention is to provide a metal injection molding feedstock composition comprising said relatively coarse stainless steel powder composition.

Another object of the invention is to provide a method for producing injection molded sintered components from the feedstock composition, said components having a density of at least 96% of the theoretical density.

Still another object of the present invention is to provide a sintered component produced according to the MIM process having a density of 96% and above, of theoretical density and a tensile strength above 800MPa as sintered, without hardening.

At least one of these objects is accomplished by:
A metal injection molding feedstock comprising
a) an iron based powder, having an median particle size of 25-45 µm, and 99% of the particles less than 120 µm, wherein the iron-based powder comprises, by weight percent; 15-17%Cr; 3-5% Ni; 3-5%,Cu; 0.15-0.45% Nb; <1.0% Mn; <1.0% Si; less than 0.08% C, balanced with Fe; and
b) 30-65% by volume of the feedstock of a binder.

The particle size is determined by laser diffraction using a Sympatec Helos instrument. The median particle size as defined above means that 50% of the particles in the powder is larger than this value. This value is normally termed the "X50" value.

A method for producing a sintered component comprising the steps of:
a) preparing a metal injection molding feedstock as suggested above;
b) molding the feedstock into an unsintered blank;
c) removing the organic binder;
d) sintering the obtained blank in a reducing atmosphere at a temperature between 1 200-1 400° C.
e) cooling the sintered component, and;
f) optionally subjecting the component to post sintering treatment such as precipitation hardening, case hardening, nitriding, carburizing, nitrocarburizing, carbonitriding, induction hardening, surface rolling and/or shot peening.

A sintered component made from the feedstock composition, the component having a density of at least 96% of theoretical density, and a tensile strength above 800MPa.

### DETAILED DESCRIPTION OF THE INVENTION

The stainless steel powder composition includes at least one iron based powder and/or pure iron powder. The iron based powder and/or pure iron powder can be produced by water or gas atomization of an iron melt and optionally alloying elements. The atomized powder can further be subjected to a reduction annealing process, and optionally be furthered alloyed by using a diffusion alloying process. Alternatively, iron powder may be produced by reduction of iron- oxides.

The particle size of the iron- or iron- based powder composition is such that the median particle size is 25-45 µm, preferably 25-35µm. Further, X₉₉ shall be at most 120µm, preferably at most 100 µm. (X₉₉ means that 99% of the particles have a particle size less than X₉₉)

Copper, Cu will enhance the strength and hardness through solid solution hardening. Cu, will also facilitate the formation of sintering necks during sintering as copper melts before the sintering temperature is reached providing so called liquid phase sintering. The powder may optionally be admixed with Cu, preferably in the form of Cu-powder in an amount of 0-5-wt%, or 3-5-wt%.

Other substances such as hard phase materials and machinability enhancing agents, such as MnS, MoS₂, CaF₂, different kinds of minerals etc. may optionally be added to the iron based powder composition.

The feedstock composition may be prepared by mixing the iron based powder composition described above and a binder.

The binder in the form of at least one organic binder may be present in the feedstock composition in a concentration of 30-65% by volume, preferably 35-60% by volume, more preferably 40-55% by volume. When using the term binder in the present description also other organic substances that are commonly in MIM-feedstocks are included, such as e.g. releasing agents, lubricants, wetting agents, rheology modifiers, dispersant agents. Examples of suitable organic binders are waxes, polyolefins, such as polyethylenes and polypropylenes, polystyrenes, polyvinyl chloride, polyethylene carbonate, polyethylene glycol, stearic acids and polyoxymethylen.

The feedstock composition is molded into a blank. The obtained blank is then heat treated, or treated in a solvent or by other means to remove one part of the binder as is known in the art, and then further subjected to sintering in a reducing atmosphere in vacuum or in reduced pressure, at a temperature of about 1200-1400°C.

The sintered component may be subjected to a heat treatment process in order to obtain a desired microstructure, e.g. by heat treatment and by controlled cooling rate. The hardening process may include known processes such as precipitation hardening, quench and temper, case hardening, nitriding, carburizing, nitrocarburizing, carbonitriding, induction hardening and the like. Alternatively, a sinter-hardening process at high cooling rate may be utilized.

Other types of post sintering treatments may be utilized, such as surface rolling or shot peening which introduce compressive residual stresses enhancing the fatigue life.

Sintered components according to the invention reach a sintered density of at least 96% of the theoretical density, and tensile strength above 800 MPa.

### EXAMPLE 1

Iron based powder compositions according to Table 1 were prepared.

**Table 1**

| **Element** | **A** | **B** | **D** | **E** | **C (comparative)** |
|---|---|---|---|---|---|
| Cr | 16.5 | 16.5 | 17 | 16.5 | 16.1 |
| Ni | 4.09 | 4.3 | 4.3 | 4.09 | 13.3 |
| Cu | 4 | 4.04 | 3.96 | 4 | |
| Nb | 0.37 | 0.37 | 0.47 | 0.37 | |
| Mn | 0.1 | 0.1 | 0.04 | 0.1 | 0.096 |
| Si | 0.68 | 0.53 | 0.95 | 0.68 | 0.881 |
| Mo | | | | | 2.12 |
| C | 0.016 | 0.079 | 0.011 | 0.016 | 0.022 |
| O | 0.351 | 0.433 | 0.146 | 0.351 | 0.236 |
| N | 0.04 | 0.025 | 0.021 | 0.04 | 0.044 |
| S | 0.007 | 0.006 | 0.003 | 0.007 | 0.009 |
| Fe | Bal | Bal | Bal | Bal | Bal |
| X10 | 10.9 | 14.2 | 14.4 | 21.4 | 12.2 |
| X50 | 24.4 | 32.6 | 31.0 | 35.0 | 26.4 |
| X90 | 46.7 | 57.0 | 52.1 | 56.7 | 46.9 |
| x99 | 72.2 | 79.8 | 86.8 | 104.0 | 66.9 |

### Example 2

The compositions were compacted to a density about 4.5g/cm³ (58% of theoretical density) into cylinders with a diameter 25mm and a height of 8mm and thereafter A, C and E were sintered at 1350°C in an atmosphere of 100%H₂ by volume, during 1200 minutes. Sample C was sintered at 1380°C, during 120 minutes, 100% H₂. Sintered density was measured using the water displacement method as described in standard SS-EN ISO 3369:2010.

**Table 2 shows the test results.**

| | **A** | **C (comparative)** | **E** |
|---|---|---|---|
| **SD** | **7.63** | **6.65** | **7.37** |
| **% of theoretical density** | **98.2** | **83.4** | **95.0** |

### Example 3

A feedstock containing the metal powder composition A, B, and D, respectively, were prepared and compared with a feedstock made from composition C, by mixing the powder compositions with an organic binder. The binder was composed of 47.5 % polyethylene, 47.5% paraffin wax and 5% stearic acid. All percentage in weight percentage. The organic binder and the powder compositions were mixed in a ratio of the metal powder:binder of 53:47 by volume.

The feedstock were injection molded into standard MIM tensile bars according to ISO- SS EN ISO 2740 The samples were then debound in hexane for 4 hours at 60°C to remove the paraffin wax, followed by sintering at 1350°C in an atmosphere of 100% hydrogen for 120 minutes.

The Sintered Density were measured using the water displacement method. Tensile test was tested according to SS EN ISO 2740. Results are shown in table 3. Standard values were taken from ISO22068 and shows values for the standard alloys 17-4PH and 316L in the sintered state. The mechanical properties are presented as % of standard value in order to be able to compare two different alloys.

**Table 3**

| | A | | B | | D | | C | |
|---|---|---|---|---|---|---|---|---|
| | Absolute value | % of standard value | Absolute value | % of standard value | Absolute value | % of standard value | Absolute value | % of standard value |
| Sintered Density (g/cm³) | 7,68 | | 7,68 | | 7,69 | | 7,38 | |
| Hardness (HRC) | 27.8 | 103 | 26.4 | 98 | 29,8 | 110 | 58.2 | 49 |
| Tensile strength (MPa) | 1129 | 141 | 1124 | 141 | 1086 | 135 | 286.5 | 64 |
| Yield strength 0.2% (MPa) | 897 | 138 | 877 | 135 | 860 | 132 | 130.9 | 94 |
| Elongation (%) | 2.9 | 97 | 2.84 | 95 | 1,4 | 47 | 22.81 | 57 |

## Claims

1. Feedstock for metal injection molding, comprising;
a) an iron based powder, having an median particle size of 25-45 µm, and 99% of the particles less than 120 µm, wherein the iron-based powder comprises, by weight percent;
15-17%Cr; 3-5% Ni; 3-5%,Cu; 0.15-0.45% Nb; <1.0% Mn; <1.0% Si; less than 0.08% C, balanced with Fe; and
b) 30-65% by volume of the feedstock of a binder.

2. Feedstock according to claim 1 wherein the binder is in the form of an at least one organic binder.

3. Feedstock according to claim 2 wherein the at least one organic binder is chosen from the group of waxes, polyolefines, such as polyethylenes and polypropylenes, polystyrenes, polyvinyl chloride, polyethylene carbonate, polyethylene glycol, stearic acids and polyoxymethylen.

4. Use of a feedstock according to any of claims 1-3 for metal injection molding.

5. A method comprising the steps of:
a) preparing a metal injection molding feedstock according to any of claims 1-3,
b) molding the feedstock into an unsintered blank,
c) removing the organic binder
d) sintering the obtained blank in a reducing atmosphere at a temperature between 1 200-1 400°C
e) cooling the sintered component, and
f) optionally subjecting the component to post sintering treatment such as precipitation hardening, case hardening, nitriding, carburizing, nitrocarburizing, carbonitriding, induction hardening, surface rolling and/or shot peening.

## Patentansprüche

1. Feedstock zum Metallpulverspritzgießen, welcher Folgendes umfasst:
a) ein Pulver auf Eisenbasis, das eine mittlere Partikelgröße von 25 bis 45 µm und 99 % der Partikel kleiner als 120 µm aufweist, wobei das Pulver auf Eisenbasis in Gewichtsprozent umfasst:
15 bis 17 % Cr; 3 bis 5 % Ni; 3 bis 5 % Cu; 0,15 bis 0,45 % Nb; < 1,0 % Mn; < 1,0 % Si; weniger als 0,08 % C, der Rest bis auf 100 % ist Fe; und
b) 30 bis 65 Vol.-% des Feedstocks eines Binders.

2. Feedstock nach Anspruch 1, wobei der Binder in Form mindestens eines organischen Binders vorliegt.

3. Feedstock nach Anspruch 2, wobei der mindestens eine organische Binder aus der Gruppe von Wachsen, Polyolefinen, wie Polyethylenen und Polypropylenen, Polystyrolen, Polyvinylchlorid, Polyethylencarbonat, Polyethylenglycol, Stearinsäuren und Polyoxymethylen ausgewählt ist.

4. Verwendung eines Feedstocks nach einem der Ansprüche 1 bis 3 zum Metallpulverspritzgießen.

5. Verfahren, welches die Schritte umfasst:
a) Herstellen eines Metallpulverspritzguss-Feedstocks nach einem der Ansprüche 1 bis 3,
b) Formen des Feedstocks zu einem ungesinterten Rohling,
c) Entfernen des organischen Binders,
d) Sintern des erhaltenen Rohlings in einer reduzierenden Atmosphäre bei einer Temperatur zwischen 1200 und 1400°C,
e) Abkühlen des Sinterformteils und
f) gegebenenfalls Unterziehen des Formteils einer Behandlung nach dem Sintern, wie z.B. Ausscheidungshärten, Einsatzhärten, Nitrieren, Aufkohlen, Nitrocarburieren, Carbonitrieren, Induktionshärten, Oberflächenwalzen und/oder Kugelstrahlen.

## Revendications

1. Charge d'alimentation pour le moulage par injection de poudre métallique, comprenant :
a) une poudre à base de fer présentant une valeur médiane de la taille des particules de 25 à 45 µm, 99 % des particules étant d'une taille inférieure à 120 µm, la poudre à base de fer comprenant, en pourcentage en poids :
15 à 17 % de Cr ; 3 à 5 % de Ni ; 3 à 5 % de Cu ; 0,15 à 0,45 % de Nb ; < 1 % de Mn ; < 1 % de Si ; moins de 0,08 % de C, le reste étant du Fe ; et
b) un liant à une teneur de 30 à 65 % en volume de la charge d'alimentation.

2. Charge d'alimentation selon la revendication 1, dans laquelle le liant se présente sous la forme d'au moins un liant organique.

3. Charge d'alimentation selon la revendication 2, dans laquelle l'au moins un liant organique est choisi dans le groupe constitué des cires, des polyoléfines, telles que les polyéthylènes et les polypropylènes, des polystyrènes, du polychlorure de vinyle, du carbonate de polyéthylène, du polyéthylèneglycol, des acides stéariques et du polyoxyméthylène.

4. Utilisation d'une charge d'alimentation selon l'une quelconque des revendications 1 à 3 pour le moulage par injection de poudre métallique.

5. Procédé comprenant les étapes consistant à :
a) préparer une charge d'alimentation de moulage par injection de poudre métallique selon l'une quelconque des revendications 1 à 3,
b) mouler la charge d'alimentation afin d'obtenir une ébauche non frittée,
c) éliminer le liant organique,
d) fritter l'ébauche obtenue dans une atmosphère réductrice à une température comprise entre 1 200 et 1 400 °C,
e) refroidir le composant fritté, et
f) soumettre éventuellement le composant à un traitement après frittage tel qu'un durcissement par précipitation, un durcissement superficiel, une nitruration, une cémentation, une nitrocarburation, une carbonitruration, une trempe par induction, un laminage superficiel et/ou un grenaillage de précontrainte.
